

## 1

3,679,590

### SOLVENT BLEACHING

Charles L. Cormany, Wadsworth, and John A. Spotts, Jr., Akron, Ohio, assignors to PPG Industries, Inc., Pittsburgh, Pa.

No Drawing. Filed Sept. 11, 1969, Ser. No. 857,214  
Int. Cl. C11d 7/54

U.S. Cl. 252—104

11 Claims

### ABSTRACT OF THE DISCLOSURE

Fabrics with both oleophilic and hydrophilic characteristics are cleansed with compositions of organic cleansing solvent throughout which an aqueous bleaching phase is dispersed. Bleaching agent remaining in the fabric is removed by a rinse solution containing the combination of an alcohol or like water soluble component and the cleansing solvent.

### BACKGROUND OF THE INVENTION

The development and increased use of cotton-polyester fabrics and the permanent press finishing of fabrics of cotton and cotton-polyester blend fabrics have created new laundering problems. These fabrics and finishes have hydrophobic tendencies. Consequently, they tend to repel water or otherwise be resistant to cleansing with conventional aqueous bleaching systems. On the other hand, traditional dry cleaning techniques, while effective with respect to oleophilic soils and stains are of little value in coping with hydrophilic stains.

Permanent press white garments such as men's shirts quite commonly encounter oleophilic soils (oils, greases, etc.) and hydrophilic soils or stains such as mustard, catsup, coffee and grape juice stains. Effective laundering must handle both categories. However, present day dry cleaning is only capable of coping with the oleophilic soils, being ineffective with respect to the hydrophilic soils. Conversely, aqueous bleaching systems designed to cope with hydrophilic stains on cotton and other hydrophilic fabrics such as linen, leave untouched oleophilic soils. Thus, neither of the two general cleaning expedients practiced by commercial laundries alone are completely satisfactory.

### THE INVENTION

This invention provides for effectively coping with both oleophilic and hydrophilic soils simultaneously and thus provides for a unitary cleansing treatment. It further provides an overall process for laundering fabrics of cotton-polyester blends and on the permanent press type which is economical and capable of being practiced in equipment appropriate for use in the commercial laundry.

According to this invention, a laundering or cleaning bath is provided which is capable of treating fabrics soiled with both oleophilic and hydrophilic stains or soils by single contact therewith. This is accomplished in accordance with the present invention by the provision of a cleaning bath which has as primary cleansing components both an organic, substantially water immiscible cleaning solvent and an aqueous phase containing a water soluble bleach. Laundering baths herein contemplated thus contain as a principal component methylchloroform, perchloroethylene, or like halogenated organic cleaning solvent along with an aqueous solution

## 2

of a water soluble bleaching agent such as aqueous hydrogen peroxide or a water soluble hypochlorite such as sodium hypochlorite. These bleaching agents are substantially insoluble in the organic cleaning solvent of the bath.

For this combination of substantially water immiscible organic cleaning solvent and aqueous solution of an organic insoluble water soluble bleaching agent to be effective, it is important these two principal components be inter-related to one another in a particular fashion. It has been discovered it is important the laundering bath include a distinct aqueous phase which constitutes a minor proportion of the bath, typically upwards of 0.1 up to 5 (rarely more than 10) percent by weight of the bath's organic cleaning solvent constituent. A distinct aqueous phase must be present contrasted with water or aqueous solution which may be dissolved in the organic cleaning solvent (even the substantially water immiscible solvents may dissolve some water).

For desirable results to accrue, the aqueous phase is dispersed throughout the organic cleaning solution phase of the bath. Distribution of the aqueous phase as a discontinuous phase through the continuous phase of organic cleaning solvent component of the bath not only insures there be proper contact between the goods and aqueous bleaching component, but prevents spot bleaching and non-uniform stain removal. As will hereinafter be further discussed, there are various sources of the water for this aqueous phase. Thus, for example, a portion of the water comprising the dispersed aqueous phase can be provided by water brought into the bath along with the materials undergoing the treatment. Without, however, a pretreating step to control the fabric's water content prior to contact with the cleansing bath of organic cleaning solvent, there is a degree of uncertainty. For this reason, recommended practices insure the presence of at least the minimum effective water content dispersed in the organic cleaning solvent of the treating bath whether or not water is introduced along with the materials subjected to the cleansing treatment.

Regardless of the source of all the water present in the cleansing composition, the water content of the bath constitutes but a minor portion of the total treating bath. This small water phase is distributed in the bath so that it contacts uniformly the material being cleansed. Small droplets of aqueous bleaching agent are thus dispersed in the continuous organic phase of the bath. Distribution of aqueous hydrogen peroxide throughout a substantially water immiscible cleaning solvent such as methylchloroform is accomplished, according to one embodiment, by use of suspending agent such as a long chain alkyl sodium phosphate. Suspending agents or surfactants facilitate dispersion of the aqueous hydrogen peroxide phase as small droplets uniformly throughout the methylchloroform even though the aqueous phase constitutes but a minor weight portion, for example, from 0.5 to 3 weight percent, of the methylchloroform.

With the aqueous hydrogen peroxide phase dispersed in the form of fine water immiscible particles, e.g., 60 globules from 1 to 500 microns, throughout the methylchloroform, the bath performs bleaching as if it was solely constituted of aqueous hydrogen peroxide, yet those fabrics treated with special advantage by the present invention (i.e., those with oleophilic and hydrophilic properties) are not degraded. By virtue of the present invention

tion, polyester-containing fabric and permanent press treated fabrics may be cleansed of both oleophilic and hydrophilic soils without significant fiber degradation.

Among other things, these ends are accomplished by restricting the contact between material and aqueous hydrogen peroxide and controlling or directing the hydrogen peroxide bleaching action. To limit the extent of the bleaching action, contact time between the peroxide and material should be controlled. Prolonged treatment, for example, on the order of several hours is definitely deteriorous to fabric strength and is also expensive. Thus, effective contact between fabric and bleaching agent, pursuant to this invention is on the order of several minutes to less than an hour, notably from 10 to 30 minutes. As will hereinafter be discussed in more detail, restricting contact times is best accomplished by use of special expedients.

A further advantage of dispersing a relatively small aqueous bleaching phase in an organic water immisible cleaning solvent is that the total amount of hydrogen peroxide or like aqueous bleaching agent required to effect the desirable level of strain removal and brightening is well below that which would be necessary in a treating bath without the organic treating solvent. In this aspect, the organic solvent acts as a distributing agent. Although diluting the bleaching agent's concentration in the bath, it does not reduce its bleaching action to a level comparable to single phase aqueous bleach bath with the same total amount of bleach agent.

The following examples illustrate the manner in which the present invention may be practiced:

#### EXAMPLE 1

A solution was prepared by passing 3600 milliliters of methylchloroform containing 29.9 grams (0.5 weight percent of methylchloroform) of Alkapent 6TD (a long chain alkyl dihydrogen phosphate sold by the Weyland Chemical Division of Philip A. Hunt Chemical Corporation) and 47.8 milliliters (1.0 percent by weight of the methylchloroform) of distilled water through 50 cubic centimeters of sodium carbonate disposed in a glass column one inch in diameter. The treatment with soda ash converted the Alkapent 6TD (a long chain alkyl dihydrogen phosphate) to long chain alkyl sodium phosphates.

From this solution a series of 150 milliliter bleach baths were provided. Ten gram scoured cotton panels were placed in the solution for two minutes, then removed. Thereafter, the specified amount of hydrogen peroxide (as 70 percent hydrogen peroxide) was rapidly added and the solution mixed. A cleaning solution thus resulted in which an immiscible aqueous hydrogen peroxide phase was dispersed in the methylchloroform. The panels were returned to the bath at room temperature (about 25° C.) for 10 minutes, and then removed, rinsed thoroughly with distilled water then acetone following which they were air dried. The panels were ironed and their blue reflectance values measured. Also, the fluidity values of the treated cloth was determined by the American Association of Textile Chemists and Colorists standard test method AATCC 82-1961.

The results are listed in Table 1.

TABLE 1

| Liquor-to-goods ratio: | Weight percent of 70% H <sub>2</sub> O <sub>2</sub> added <sup>1</sup> | Blue reflectance, percent | Cuam fluidity (rhes) |
|------------------------|------------------------------------------------------------------------|---------------------------|----------------------|
| 20:1                   | 5                                                                      | 71.9                      | 3.0                  |
| 20:1                   | 10                                                                     | 74.6                      | 3.0                  |
| 20:1                   | 15                                                                     | 74.8                      | 3.0                  |
| 20:1                   | 20                                                                     | 75.6                      | 3.0                  |
| 20:1                   | 25                                                                     | 80.6                      | 3.4                  |
| 20:1                   | 30                                                                     | 81.2                      | 3.4                  |
| No treatment           |                                                                        | 55.7                      | 3.4                  |

<sup>1</sup> By weight of cotton panels.

#### EXAMPLE 2

A stock solution was prepared by adding 3.4 grams of sodium carbonate dissolved in 20 milliliters of distilled water to 3 liters of methylchloroform containing 10 grams (0.5 weight percent of the methylchloroform) of Alkapent 6TD. Amounts of 70 percent hydrogen peroxide (as specified in Table 2) were added to 150 milliliter samples of this stock solution. Ten grams scoured cotton panels were placed in the baths at room temperature for 10 minutes and removed, rinsed in distilled water, air dried and ironed, following which the blue reflectance was measured with these results:

TABLE 2

| Weight percent <sup>1</sup> of 70% H <sub>2</sub> O <sub>2</sub> used: | Blue reflectance, percent |
|------------------------------------------------------------------------|---------------------------|
| 1.3                                                                    | 70.2                      |
| 2.6                                                                    | 72.5                      |
| 6.4                                                                    | 74.5                      |
| 7.7                                                                    | 74.6                      |
| 10.0                                                                   | 76.7                      |
| 13.0                                                                   | 77.0                      |

<sup>1</sup> By weight of the cotton panel.

Contact between the fabric and the cleaning solution is relatively brief; contact for as little as about 5 minutes to 30 or 40 minutes achieve a high degree of bleaching. This is illustrated by the following examples:

#### EXAMPLE 3

A stock solution was prepared by passing three liters of methylchloroform containing 20 grams of Alkapent 6TD (0.5 percent by weight of the methylchloroform) and 40 milliliters of distilled water through a bed of sodium carbonate. The sodium carbonate treatment converted the Alkapent 6TD (long chain alkyl dihydrogen phosphate) to a long chain alkyl sodium and disodium phosphate. Ten grams scoured cotton panels were then placed for the specified period of time in 150 milliliter portions of the bleach liquor to which the amounts of 70 percent hydrogen peroxide specified in Table 3 had been added and then removed, water washed, air dried and ironed. The reflectance and fluidity of many of these samples were determined and are reported in Table 3. Without the treatment, the cotton had a blue reflectance of 64.7 percent and a Cuam fluidity of 2.2 rhes.

TABLE 3

| Concentration of 70% H <sub>2</sub> O <sub>2</sub> (OWG) <sup>1</sup> percent | Blue reflectance, percent | Cuam fluidity (rhes) |
|-------------------------------------------------------------------------------|---------------------------|----------------------|
| Time (minutes):                                                               |                           |                      |
| 5                                                                             | 69.2                      | 3.0                  |
| 10                                                                            | 70.2                      | 3.2                  |
| 15                                                                            | 72.3                      | 3.5                  |
| 20                                                                            | 74.1                      | 3.4                  |
| 30                                                                            | 75.2                      | 4.1                  |
| 5                                                                             | 70.3                      | 2.7                  |
| 10                                                                            | 73.1                      | 3.3                  |
| 15                                                                            | 75.0                      | 3.6                  |
| 20                                                                            | 76.2                      | 3.8                  |
| 30                                                                            | 79.2                      | 4.7                  |
| 5                                                                             | 71.8                      | 3.2                  |
| 10                                                                            | 74.6                      | 3.5                  |
| 15                                                                            | 76.8                      | 3.9                  |
| 20                                                                            | 76.5                      | 4.3                  |
| 30                                                                            | 79.2                      | 5.0                  |
| 5                                                                             | 72.7                      |                      |
| 10                                                                            | 76.3                      | 3.1                  |
| 15                                                                            | 77.2                      | 3.7                  |
| 20                                                                            | 78.2                      | 3.7                  |
| 30                                                                            | 80.0                      | 4.5                  |
| 5                                                                             | 73.9                      | 2.6                  |
| 10                                                                            | 76.8                      | 3.3                  |
| 15                                                                            | 77.4                      | 3.3                  |
| 20                                                                            | 79.5                      | 3.6                  |
| 30                                                                            | 80.3                      | 4.4                  |

<sup>1</sup> OWG=On the weight of the goods.

#### EXAMPLE 4

The procedure of Example 3 was repeated with three different levels of hydrogen peroxide. The cotton without bleaching had a Blue Reflectance of 65.7 percent and a Cuam fluidity of 2.2 rhes.

The following Table 4 lists the data:

TABLE 4

| Time (minutes): | Concen-<br>tration of<br>70% H <sub>2</sub> O <sub>2</sub><br>(OWG),<br>percent | Blue<br>reflec-<br>tance,<br>percent | Cuam<br>fluidity<br>(rhe) |
|-----------------|---------------------------------------------------------------------------------|--------------------------------------|---------------------------|
| 2               | 3.2                                                                             | 68.4                                 | -----                     |
| 4               | 3.2                                                                             | 69.3                                 | -----                     |
| 6               | 3.2                                                                             | 71.2                                 | 2.9                       |
| 8               | 3.2                                                                             | 72.4                                 | 2.9                       |
| 10              | 3.2                                                                             | 72.9                                 | -----                     |
| 20              | 3.2                                                                             | 74.7                                 | -----                     |
| 30              | 3.2                                                                             | 75.4                                 | 3.3                       |
| 60              | 3.2                                                                             | 77.7                                 | 3.4                       |
| 2               | 6.4                                                                             | 71.2                                 | -----                     |
| 4               | 6.4                                                                             | 71.1                                 | -----                     |
| 6               | 6.4                                                                             | 72.6                                 | -----                     |
| 8               | 6.4                                                                             | 74.1                                 | -----                     |
| 10              | 6.4                                                                             | 75.7                                 | 2.5                       |
| 20              | 6.4                                                                             | 78.8                                 | -----                     |
| 30              | 6.4                                                                             | 78.5                                 | 3.0                       |
| 60              | 6.4                                                                             | 80.8                                 | 3.4                       |
| 5               | 10.0                                                                            | 72.3                                 | -----                     |
| 15              | 10.0                                                                            | 77.4                                 | -----                     |
| 20              | 10.0                                                                            | 78.6                                 | -----                     |
| 30              | 10.0                                                                            | 78.8                                 | 2.4                       |

<sup>1</sup> OWG=On the weight of the goods.

EXAMPLE 5

A stock solution of bleach bath compositions for the first four runs reported in Table 5 was prepared by adding 0.17 gram of sodium carbonate in water of 150 milliliters of methylchloroform composition which contained 0.5 weight percent of Alkapent 6TD, the amount of water used to dissolve the sodium carbonate being 0.5, 1.0, 1.5 and 2.0 milliliters respectively. The remaining three runs used a stock solution provided by adding 1.8 grams of sodium carbonate dissolved in 5 milliliters of water to 750 milliliters of methylchloroform containing 0.5 weight percent Alkapent 6TD. Additionally, 1.0 milliliter and 2.0 milliliters of water were added respectively to the last two samples. A quantity of 70 percent hydrogen peroxide (0.78 milliliter) was added to each 150 milliliter portion. The ten-gram scoured cotton panels were then in the solvent for 10 minutes, the panels removed, rinsed with distilled water, air dried and ironed.

TABLE 5

| Water<br>concentration <sup>1</sup><br>percent | Blue<br>reflec-<br>tance,<br>percent | Cuam<br>fluidity<br>(rhe) |
|------------------------------------------------|--------------------------------------|---------------------------|
| (OWG) <sup>2</sup> (OWS) <sup>3</sup>          | percent                              | (rhe)                     |
| 5                                              | 0.25                                 | 74.1                      |
| 10                                             | 0.5                                  | 75.3                      |
| 15                                             | 0.75                                 | 75.2                      |
| 20                                             | 1.0                                  | 74.5                      |
| 20                                             | 1.0                                  | 75.2                      |
| 30                                             | 1.5                                  | 75.4                      |
| 40                                             | 2.0                                  | 75.2                      |
|                                                |                                      | 3.2                       |

<sup>1</sup> Exclusive of water added as 70% H<sub>2</sub>O<sub>2</sub>.

<sup>2</sup> OWG=By weight of the cotton goods.

<sup>3</sup> OWS=By weight of the methylchloroform.

As noted, the cleansing solution includes a suspending agent which serves to facilitate and maintain the aqueous bleaching phase in the desirable dispersed state. In many instances, besides performing this important function, these agents facilitate the bleaching action of the agent. Many are also detergents (as well as suspending agents) and hence their presence adds this to the cleansing capacity of the treating solution. Most are either anionic or nonionic.

Any one of many suspending agents work as evidenced by the examples. In addition, these may be mentioned: octyl phenoxy polyethoxy ethanol (nonionic), polyethylene glycol ester of oleic acid (nonionic), nonyl phenyl polyethylene glycol ether (nonionic), nonyl phenoxy poly(ethyleneoxy) ethanol (nonionic), polyoxyethylene polyol fatty acid esters (nonionic), sodium dodecyl diphenyl ether disulfonate (anionic), octyl phenoxy polyethoxy ethanol (nonionic), alkylaryl polyether alcohol (nonionic), octyl phenoxy ethanol (nonionic) and octyl phenoxy diethoxy ethanol (nonionic).

An important consideration is timely and complete removal of active bleaching agent, notably active hydrogen peroxide from the treated fabric. Fabrics of the type most appropriately treated by this invention lose strength if they retain hydrogen peroxide (or like bleaching agent). Overcontact with bleaching agent is detrimental to fabric strength. It has been found that even such minor amounts of residual bleaching agent which remain in the fabric can cause serious fabric degradation. Detrimental amounts of hydrogen peroxide and the like are retained by the fabric even after the fabric is withdrawn from the treating bath and solvent rinsed by normal expedients.

According to an embodiment of this invention, a particularly effective means for removing residual hydrogen peroxide and thereby preventing fiber degradation has been developed. Various attempts to use components of the cleaning bath for removal of hydrogen peroxide did not prove effective as illustrated by Example 6.

## EXAMPLE 6

Ten gram scoured cotton panels were treated for 10 minutes at room temperature in a cleansing bath provided by passing 150 milliliters of methylchloroform containing one gram of Alkapent 6TD and two grams of distilled water through a sodium carbonate column to which was added 2.34 milliliters of 70 percent hydrogen peroxide. Thereafter, the panels were rinsed as described in Table 6 and the Blue Reflectance and fluidity of the panels measured:

TABLE 6

| Run | Type of rinse treatment                                                                                          | Blue<br>reflec-<br>tance,<br>percent | Cuam<br>fluidity<br>(rhe) |
|-----|------------------------------------------------------------------------------------------------------------------|--------------------------------------|---------------------------|
| 35  | (1) Water                                                                                                        | 79.4                                 | 8.0                       |
|     | (2) Three consecutive rinses with methylchloroform                                                               | 79.9                                 | 15.4                      |
|     | (3) Same as (2) but with 0.05% alkaline Alkapent 6TD and 1.0% H <sub>2</sub> O <sub>2</sub>                      | 80.8                                 | 17.6                      |
| 40  | (4) Rinse once with the composition of (3) followed by rinse (2)                                                 | 80.1                                 | 10.3                      |
|     | (5) Same as (4) except that the 0.05% formic acid included in the composition of (3)                             | 80.9                                 | 18.4                      |
|     | (6) Rinsed twice with methylchloroform containing acidic Alkapent 6TD followed by two rinses of methylchloroform | 79.5                                 | 12.4                      |

In each of these runs, fiber degradation progressed further than desirable, as evidenced by the high Cuam fluidity values.

Residual hydrogen peroxide or like bleaching agent, it has been discovered, is reduced to a tolerably low level (i.e., to a level at which serious fiber degradation is avoided) in the treated fabric by rinsing the fabric with a special formulation containing as basic constituents an organic cleaning solvent, ideally the same organic solvent employed in the cleaning step, along with a minor concentration of a substantially water soluble alcohol. Such alcohols include monohydric aliphatic alcohols such as ethanol, isopropanol, n-propanol, t-butanol, isobutanol, the amyl alcohols such as t-amyl alcohol, and the like, notably, alkanols containing from 2 to 5 carbon atoms. Useful alcohol concentrations in the rinse compositions are from 1 to 10 percent or even 15 percent by volume of the organic cleansing solvent. Preferably, monohydric alcohols should have a substantial miscibility in both the organic cleaning solvent and in water, so that in the concentrations it is present it will not form (or cause to form) a second distinct liquid phase. It is desirable that the rinse composition before and after use be as a single liquid phase. Alcohols with a relatively low boiling point (below about 100° C.) are advantageous; they are readily removed from the fabric by those drying procedures normally utilized in connection with the cleaning of fabrics in commercial laundry operations.

Where the concentration of the alcohol creates fire hazards or other disadvantages, a monoether of a dihydric compound, notably, lower alkyl monoethers of glycols such as methyl Cellosolve, ethyl ether or glycol, and like water soluble, organic soluble monoether can be included in the rinse formulation. This permits a reduction in the alkanol without hampering the composition's performance.

Other materials useful in lieu of or in addition to the alcohols and ethers already described include dioxane, ketones such as acetone and methyl ethyl ketone, etc.

Rinse compositions will also contain a small amount of water. For one thing, residual water from the treated fabric will find its way into the rinse. As hereinafter discussed, use as by recycle is contemplated of rinse solution which has previously been in contact with treated fabric. Water contents range from about 0.1 to 5 weight percent, of the organic solvent, or sometimes even higher (e.g., up to about 10 percent). It is preferred practice for the water content to be below that which will give rise to a separate (immiscible aqueous) phase; ergo, the water is present as dissolved water. A separate liquid phase of any kind presents complications in the adaption of more common dry cleaning equipment to this method and hence is better avoided.

Other expedients reduce residual hydrogen peroxide in the fabric. For example, residual hydrogen peroxide may in effect be removed by contact with a material with which it reacts. Various reagents which reduce hydrogen peroxide are thus of use. Some such reagents include inorganic reducing agents such as ferrous ammonium sulfate, sodium sulfite, sodium bisulfite, potassium sulfite, potassium bisulfite, ammonium sulfate, ammonium bisulfite and organic reducing agents exemplified by thioureas such as allyl thiourea diethylthiourea and dibutylthiourea; aldehydes such as formaldehyde, pyruvaldehyde and glycidaldehyde.

In using these reducing agents to remove bleaching agent, it is advisable to rinse the fabric free of products (salts) of the reduction of hydrogen peroxide. Often those salts can cause discoloration or odor, even as such, or after further treatment of the fabric. Ironing or other heating will often result in discoloration with some of the salts. Water soluble salts, for example, may be water rinsed away. Organics can be dissolved in an appropriate organic rinse.

#### EXAMPLE 7

Cotton fabric was treated for 10 minutes at room temperature in a bath of methylchloroform containing 0.5 percent Triton GR-7 (a Rhone & Haas product; diethyl sodium sulfosuccinate) anionic suspending agent and by weight of the fabric, 30 percent water, 4.5 percent ammonium hydroxide and 10 percent of 70 percent hydrogen peroxide. After being withdrawn from the bleaching bath, the fabric was contacted for 9 minutes with sixty weight parts per part of fabric of a liquid composition of methylchloroform containing 0.5 weight percent of Triton GR-7 the solvent and (by weight of the fabric) 20 percent water, and 7 percent sodium sulfite. Three one-minute methylchloroform rinses followed. Residual hydrogen peroxide in the fabric was 0.19 percent.

The following examples illustrate rinsing techniques for reducing residual hydrogen peroxide on fabrics which have been cleansed by treatment with a bath of an organic cleansing solvent through which a dispersed aqueous water soluble bleach containing phase is dispersed uniformly.

#### EXAMPLE 8

In each of the tests, a ten gram neutral scoured cotton panel was bleached for 10 minutes at room temperature in 150 milliliters of methylchloroform composition to which 0.5 gram of Alkapent 6TD, 0.5 milliliter of distilled

water, 0.085 gram of sodium carbonate and 0.5 milliliter of 70 percent hydrogen peroxide had been added. The panels were then removed, hand squeezed, dried and rinsed with the compositions and in the manner described in Table 7.

Following the rinsing, a 5 gram portion of the cotton panel was tested to determine its residual hydrogen peroxide content.

Unless otherwise indicated, each rinse was for two minutes, the volume of rinse material was 250 milliliters and six rinses were employed.

TABLE 7

| Run No. | Rinse bath Additive               | Volume percent | Quantity of H <sub>2</sub> O <sub>2</sub> remaining in fabric, percent OWG | Blue reflectance percent | Cuam fluidity (rhes) |
|---------|-----------------------------------|----------------|----------------------------------------------------------------------------|--------------------------|----------------------|
| Control |                                   |                | 3.22                                                                       |                          |                      |
| 1       | 2-propanol                        | 5              | 0.62                                                                       |                          |                      |
| 2       | do                                | 10             | 0.31                                                                       | 73.6                     | 3.7                  |
| 3       | Dioxane                           | 5              | 1.31                                                                       |                          |                      |
| 4       | Quinoline                         | 5              | 0.68                                                                       |                          |                      |
| 5       | 2-methyl-1-propanol               | 10             | 0.56                                                                       |                          |                      |
| 6       | (2-propanol) <sup>1</sup> (Water) | 10 } 20.3 }    | 0.08                                                                       |                          |                      |
| 7       | (2-propanol) <sup>2</sup> (Water) | 10 } 20.6 }    | 0.19                                                                       |                          |                      |
| 8       | 2-propanol <sup>3</sup>           | 10             | 0.22                                                                       |                          |                      |
| 9       | (2-propanol) <sup>4</sup> (Water) | 10 } 0.3 }     | 0.03                                                                       | 74.6                     | 3.7                  |

<sup>1</sup> Fabric after bleaching.

<sup>2</sup> Percent by weight of methylchloroform.

<sup>3</sup> 50/50 Dacron/cotton panels with permanent press resin finish treatment.

<sup>4</sup> Rinse volumes of 150 milliliters.

#### EXAMPLE 9

A ten gram neutral cotton panel was treated for 10 minutes at room temperature with 150 milliliter portions of a stock solution prepared by adding 1.7 grams of sodium carbonate, 10 grams of Alkapent 6TD and 10 milliliters of distilled water to 3,000 milliliters of perchloroethylene and to which portion 0.5 milliliter of 70 percent hydrogen peroxide was added. After removal from the treating bath, the panel was rinsed six times using each time 250 milliliters of a perchloroethylene rinse composition containing 10 percent by volume 2-propanol and 1 milliliter of distilled water. Following this rinsing, the panel was dried in a forced air oven at about 70° C. until all solvent vapors had been expelled, then ironed. Its residual hydrogen peroxide content was 0.09 percent and it had a Cuam fluidity of 3.8 rhes.

Removal of stains by the cleansing composition of this invention is illustrated in the following examples.

#### EXAMPLE 10

Samples of fabric each with mustard, ball point ink, grape juice, coffee or chocolate milk stains were prepared and then placed for 20 minutes at room temperature in a bleach bath of methylchloroform to which had been added (by weight of the methylchloroform) 6.5 percent of 70 percent hydrogen peroxide, 0.85 percent sodium carbonate, 5.0 percent water and by weight percent of the goods 0.25 percent Alkapent 6TD, the amount of such bleach bath providing a 20:1 weight ratio of solvent to goods.

The fabrics were then removed, their residual hydrogen peroxide destroyed, and their reflectances determined with these results:

TABLE 8

| Stain                       | Initial reflectance, percent |                   | Final reflectance, percent |                   | 15   |      |
|-----------------------------|------------------------------|-------------------|----------------------------|-------------------|------|------|
|                             | Blue                         |                   | Green                      |                   |      |      |
|                             | Inc. <sup>1</sup>            | Exc. <sup>2</sup> | Inc. <sup>1</sup>          | Exc. <sup>2</sup> |      |      |
| 100% COTTON FABRICS         |                              |                   |                            |                   |      |      |
| Mustard.....                | 37.4                         | 36.9              | 79.2                       | 60.0              | 58.8 | 85.4 |
| Coffee.....                 | 43.4                         | 43.5              | 62.1                       | 61.7              | 61.9 | 74.3 |
| Ink.....                    | 77.2                         | 77.3              | 57.7                       | 81.9              | 81.6 | 84.7 |
| Grape juice.....            | 27.9                         | 26.6              | 45.5                       | 56.9              | 56.9 | 75.2 |
| Chocolate milk.....         | 56.7                         | 56.6              | 69.4                       | 66.0              | 64.3 | 75.4 |
| 50/50 DACRON-COTTON FABRICS |                              |                   |                            |                   |      |      |
| Mustard.....                | 50.1                         | 45.9              | 77.1                       | 68.4              | 60.0 | 80.6 |
| Coffee.....                 | 43.6                         | 37.9              | 58.5                       | 73.2              | 65.4 | 77.6 |
| Ink.....                    | 84.6                         | 73.7              | 65.3                       | 87.5              | 76.4 | 79.9 |
| Grape juice.....            | 39.6                         | 36.4              | 50.6                       | 82.4              | 72.3 | 80.4 |
| Chocolate milk.....         | 62.9                         | 55.1              | 69.5                       | 81.5              | 71.7 | 79.9 |

<sup>1</sup> Inc. = Including fluorescence.

<sup>2</sup> Exc. = Excluding fluorescence.

Organic cleaning solvents other than methylchloroform, as exemplified by the use of perchloroethylene in Example 9, are effective. Usually these cleaning solvents are essentially water immiscible. The more notable are halogenated hydrocarbon solvents, having 1 to 3 carbons. Besides methylchloroform these include chloroform, carbon tetrachloride, methylene chloride, methylene dichloride, ethylene dichloride, trichloroethylene, perchloroethylene, many of their fluorinated or chlorofluorocounterparts such as 1,1,2-trifluoro 1,2,2-trichloroethane, difluoromethane, trifluoroethylene, chloro-fluoro hydrocarbon cleaning solvents, such as trichlorofluoromethane, 1,1,2,2-tetrafluoro 1,2-dichloroethane, as well as other halogenated solvents containing two or more different halogens. Other solvents include petroleum dry cleaning solvents such as the Stoddards Solvents.

Example 11 illustrates applicability of halogen bearing organic cleaning solvents.

#### EXAMPLE 11

The general procedure involved treating with a cleansing bath provided by mixing about 0.5 millimeter of 70 percent hydrogen peroxide into 150 milliliters of a solution provided by adding 0.55 gram of Alkapent 6TD and 0.5 millimeter of 3.2 Normal sodium carbonate to the organic solvent. A ten gram sample of 100 percent scoured cotton was placed in the bath at room temperature and agitated for 10 minutes. The bath composition and liquor-to-goods ratio in the treatment was such that the hydrogen peroxide content of the bath was 6.4 percent, the sodium carbonate was 0.85 percent, the water constituted 5 percent (all by weight of the organic cleaning solvent) and the Alkapent 6TD content was 0.25 percent by weight of the goods.

Following the cleansing treatment, the fabric from each cleansing step was then treated for 5 minutes at 25° C. in a bath of the solvent employed in the cleansing step containing sodium sulfite ( $Na_2SO_3$ ), a small amount of water and about 1 gram of Triton GR-7 (an anionic neutral detergent). The sodium sulfite reacted with residual hydrogen peroxide in the fabric.

The fabric was then placed in the bath of the solvent containing a small amount of dilute hydrochloric acid and about 1 gram of Triton GR-7 for the purpose of destroying any salts generated by the sulfite. Then it was rinsed with solvent only to remove any residual Triton GR-7 following which the sample was air dried for three minutes and then ironed. Samples ironed to dryness had their reflectance values determined.

The following Table 9 tabulates the results:

TABLE 9

| 5                                           | Solvent | Blue reflectance, percent | Cuam fluidity (rhees) |
|---------------------------------------------|---------|---------------------------|-----------------------|
| Perchloroethylene.....                      | 74.0    | 3.8                       |                       |
| Chloroform.....                             | 73.6    | 3.2                       |                       |
| 1,1,2-trichloro, 1,2,2-trifluoroethane..... | 73.3    | 2.9                       |                       |
| Methylene chloride.....                     | 73.9    | 2.9                       |                       |
| Carbon tetrachloride.....                   | 75.8    | 3.1                       |                       |
| Ethylene dichloride.....                    | 73.1    | 4.3                       |                       |
| Trichloroethylene.....                      | 72.1    | 4.0                       |                       |

In lieu of hydrogen peroxide as the bleaching component of the cleansing or organic solvent bleaching system, other water soluble bleaches may be employed, especially those water soluble bleaches which are substantially insoluble in the organic cleaning solvent of the cleaning bath. Besides hydrogen peroxide, alkali metal peroxides such as sodium peroxide, hypochlorous acid and the alkali hypochlorites such as sodium hypochlorite, potassium hypochlorite and lithium hypochlorite as well as mixtures of one or more (including hydrogen peroxide) are effective.

Typical practice of the invention herein described utilizing equipment of the type available to and in the commercial laundry involves charging a dry cleaning wheel with soiled garment following which the cleansing composition (of the invention) is then introduced into the wheel. The fabric is agitated in the cleaning solvent usually for from 5 to 25 minutes whereupon the solvent is drained promptly from the wheel and the garments therein extracted (spin dried), a typical time period for this being from 2 to 5 minutes.

Once the garments are freed of extraneous cleansing solvent, they are rinsed with a solution comprised of the organic cleaning solvent (utilized in the cleaning step), a minor amount of monohydric alcohol such as isopropyl alcohol alone or in combination with methyl-Cellosolve and a small amount of water. Effective results are obtained when the rinse solution is continuously circulated through and out of the dry cleaning wheel. The monohydric constituents should be present in a quantity sufficient to dissolve the hydrogen peroxide from the fabric and also avoid the formation of separate immiscible phase in the circulating rinse solution. It especially is important to maintain the rinse solutions as a single liquid phase when the circulating solution is passed through filters (for purification) designed to handle but a single liquid phase, a typical characteristic of filter systems in many dry cleaning apparatus.

Residual hydrogen peroxide in the garments is reduced with particular effectiveness by continuously removing rinse solution from the wheel, destroying or reducing the peroxide content of the solution, and returning it to the wheel. Contacting the rinse composition with materials which selectively decompose hydrogen peroxide will accomplish this. Typically, polyvalent metals are of use in this connection. Palladium deposited on a particulate clay substrate, for example, provides an excellent bed through which to pass the rinse solution for the purpose of destroying hydrogen peroxide. Other metals useful in lieu of palladium include silver, platinum, ruthenium, manganese and the like. In general, those polyvalent metals which do not form oxides soluble in the rinse solution are preferred since soluble oxides dissolve and accumulate, and ultimately will have to be removed from the system. Ferromanganese alloys, silver oxide, activated carbon, cobalt chloride impregnated on calcium sulfate are among many other useful materials.

Upon freeing the garment's residual hydrogen peroxide, any residual rinse solvent is drained from the fabrics usually in less than 5 or 10 minutes. The garments are then dried by a typical procedure employed in dry cleaning, notably by contact with hot air for several minutes. Solvent vapors in the hot air are usually removed by con-

dersation from the hot air exiting the dry cleaning wheel. Other steps used in dry cleaning may be performed such as deodorizing.

EXAMPLE 12

Use of a commercial type short cycle dry cleaning unit with some adaptation in materials of construction (e.g., use of polyethylene tubing in lieu of rubber hosing) and provision of two tanks for handling two different liquid compositions demonstrated the applicability of the system to commercial equipment as follows.

Cleansing solution was provided by adding 0.38 pound of Alkaptent 6TD, 29.4 grams sodium carbonate monohydrate in 199 milliliters of distilled water and 260 milliliters of 35 percent hydrogen peroxide to 14 gallons of methylchloroform. Eight gallons of this solution was fed to the dry cleaning wheel which contained five (5) pounds of fabric (of the type identified in the table). Then 260 milliliters of 35 percent hydrogen peroxide was added, whereafter the fabric and solvent were agitated in the wheel for 20 minutes at room temperature and the liquid drained from the wheel in three minutes.

Rinsing was then commenced by circulating several gallons per minute of a methylchloroform solution containing 5 volume percent (2.15 gallons) isopropanol, 2 volume percent (1.02 gallons) methylcellosolve and 0.25 volume percent (0.122 gallon) water for 25 minutes at room temperature through the dry cleaning wheel. As it is recirculated, the rinse composition withdrawn from the wheel was passed through a cartridge of finely divided clay impregnated with two weight percent palladium. This catalyzed decomposition of hydrogen peroxide so that rinse solvent returned to the wheel was depleted of hydrogen peroxide. As a result, the residual hydrogen peroxide in the fabric was substantially removed.

Then the wheel contents were rinsed and extracted of liquid in three minutes, following which hot air drying was conducted for seven minutes.

These results were obtained:

TABLE 10

| Fabric              | Percent          |                   |           |
|---------------------|------------------|-------------------|-----------|
|                     | Blue reflectance | Green reflectance | Whiteness |
| Scoured cotton:     |                  |                   |           |
| Before <sup>1</sup> | 66.5             | 74.2              | 43.4      |
| After               | 82.3             | 87.4              | 67.0      |

<sup>1</sup> As placed in wheel.

EXAMPLE 13

The general procedure and apparatus of Example 12 was duplicated with certain changes. The initial cleansing composition contained 8 gallons of 0.19 percent sodium hypochlorite rather than hydrogen peroxide. After 5 minutes treatment with this composition, 40.5 milliliters of 35 percent hydrogen peroxide was added and the treatment continued for 5 minutes followed by draining and extraction of the cleansing solution. Rinsing in this procedure was for 15 minutes.

These results were obtained:

TABLE 11

| Fabric               | Percent          |                   |           |
|----------------------|------------------|-------------------|-----------|
|                      | Blue reflectance | Green reflectance | Whiteness |
| Scoured cotton:      |                  |                   |           |
| Before               | 65.4             | 72.8              | 43.2      |
| After                | 81.8             | 87.4              | 65.0      |
| After <sup>1</sup>   | 82.1             | 86.9              | 67.7      |
| 50/50 dacron-cotton: |                  |                   |           |
| Before               | 79.5             | 84.7              | 63.9      |
| After                | 82.4             | 88.1              | 65.3      |
| After <sup>1</sup>   | 84.7             | 87.4              | 76.6      |

<sup>1</sup> Use of fabric once treated.

In practice, cleaning solvent extracted from the dry cleaning wheel and the cleaning step of the process is collected in an appropriate storage container. So too, the

rinse solution. Prior to further use with a fresh charge of soiled garments, the solution is replenished with the additional aqueous bleaching material such as hydrogen peroxide.

5 Special techniques are useful when the aqueous component of the cleansing compositions is other than hydrogen peroxide. For example, with aqueous sodium hypochlorite or the like, it is especially beneficial to combine the use of sodium hypochlorite with hydrogen peroxide. Thus, in one contemplated procedure, the goods are initially treated with an organic cleansing solution in which the aqueous bleach phase is aqueous sodium hypochlorite for a short period of time, say 3 to 15 minutes. Then, hydrogen peroxide is added and a further cleansing action is effected. This sequence of aqueous bleaching agents provides a unique combination of the particularly effective qualities of each. In addition, by utilizing the hydrogen peroxide step last, only hydrogen peroxide is left in the fabric. It can be removed by treatment with the alcohol containing solvent rinse solution.

20 Techniques herein described are especially applicable to the cleansing of fabrics (or garments of fabrics) which possess both oleophilic and hydrophilic characteristics and hence are soiled (or stained) by both oleophilic and hydrophilic soils. In general, such garments are primarily cotton-polyester blends. The so-called white goods of such fabrics are advantageously treated. Colored fabrics whose dyes are set by oxidizing reaction also are treated with facility, the oxidizing action of the aqueous bleach revitalizing the dye color. Of course, those dyes which are detrimentally effected by aqueous bleach materials are less readily susceptible of this treatment. Nevertheless, because exposure to the aqueous peroxide phase is controlled, it is possible to treat colored fabric quite often without intolerable color degradation.

25 Temperatures of treatment in each of the steps herein discussed are those normally encountered in cleaning operations. Ergo the process can be effectively used without recourse to unusual conditions of pressure or temperature.

30 While the present invention has been described with respect to certain details of special embodiments, it is not intended that the invention be construed as limited thereto except and insofar as details are set forth in the claims.

We claim:

35 1. A method of treating fabric which comprises contacting the fabric with a cleaning bath having as its principal components a continuous phase of substantially water immiscible organic cleaning solvent which constitutes a major portion of the bath and having dispersed therein and constituting a minor portion of the bath, a discontinuous distinct aqueous bleaching phase substantially immiscible in the organic cleaning solvent of a water soluble bleaching agent which bleaching agent is substantially insoluble in the water immiscible organic cleaning solvent of the continuous phase, terminating contact between the fabric and cleaning bath before serious fabric degradation due to the bleaching agent occurs and removing residual bleaching agent remaining in the fabric by rinsing the fabric with a substantially water immiscible organic cleaning solvent having a minor amount of a 2 to 5 carbon monohydric alcohol.

40 2. The method of claim 1 wherein the solvent is a 1 to 3 carbon halogenated hydrocarbon and the bleaching agent in the bleaching phase is selected from the group consisting of hydrogen peroxide, alkali metal peroxides, hypochlorous acid and alkali metal hypochlorites.

45 3. A method of treating fabric which comprises contacting the fabric with a two phase cleaning bath having an organic suspending agent and as its principal components a continuous phase of substantially water immiscible organic 1 to 3 carbon chlorinated hydrocarbon cleaning solvent constituting a major portion of the bath having dispersed therein and constituting a minor portion of the bath a distinct discontinuous aqueous bleaching phase substantially immiscible in the organic cleaning solvent of a water soluble bleaching agent selected from

the group consisting of hydrogen peroxide, alkali metal peroxides, hypochlorous acid and alkali metal hypochlorites, terminating contact between fabric and cleaning bath before serious fabric degradation due to the bleaching agent occurs and removing residual bleaching agent remaining in the fabric from said treatment by rinsing the fabric with a single liquid phase rinse of the same organic cleaning solvent used in cleaning having a minor concentration of a 2 to 5 carbon monohydric alkanol.

4. A method of treating fabric with both oleophilic and hydrophilic characteristics which comprises contacting the fabric with a two phase cleaning composition having as principal components a continuous phase of substantially water immiscible organic halogenated hydrocarbon cleaning solvent throughout which is dispersed a distinct aqueous organic immiscible phase of a water soluble bleaching agent, which bleaching agent is substantially insoluble in the organic halogenated hydrocarbon cleaning solvent of the continuous phase, said dispersed distinct aqueous phase constituting from 0.1 to 10 percent by weight of the cleaning solvent in the continuous phase, separating the fabric from contact with the composition before significant fabric degradation occurs and promptly removing residual bleaching agent in the fabric by rinsing the fabric with organic substantially water immiscible cleaning solvent which has a minor portion of a 2 to 5 carbon monohydric alkanol.

5. The method of claim 4 wherein the cleaning composition also has a long chain alkyl sodium phosphate, the solvent is selected from the group consisting of methylchloroform, perchloroethylene and trichloroethylene and the bleaching agent is selected from the group consisting of hydrogen peroxide, alkali metal peroxides, hypochlorous acid and alkali metal hypochlorites.

6. The method of claim 4 wherein residual water soluble bleaching agent remaining in the fabric after separation from the cleaning composition is removed by rinsing the fabric with a liquid rinse of the organic cleaning solvent having from 1 to 15 percent by volume of said organic cleaning solvent of a 2 to 5 carbon monohydric alkanol.

7. The method of claim 6 wherein the rinse composition also has a small amount of a water soluble, lower

alkyl monoether of a glycol soluble in the organic solvent of the rinse composition.

8. A method of removing residual water soluble bleaching agent from a fabric containing residual bleaching agent from a cleansing treatment in which the fabric has been contacted with the water soluble bleaching agent which comprises rinsing the fabric with a rinse composition of a substantially water insoluble organic cleaning solvent containing dissolved therein a minor concentration of a 2 to 5 carbon monohydric alkanol.

9. The method of claim 8 wherein the bleaching agent removed from the fabric during the rinsing and present in the rinsing solution is destroyed by contacting the solution with an inorganic decomposition catalyst for destroying the bleaching agent and thereafter contacting the fabric further with the rinse composition which has had bleaching agents present so decomposed.

10. The method of claim 8 wherein the alkanol concentration in the rinse composition is from 1 to 15 percent by volume of the organic cleaning solvent, and the rinse composition includes a water soluble lower alkyl ether of a glycol which is also soluble in the organic cleaning solvent.

11. The method of claim 8 wherein the rinse composition is a single liquid phase and contains water in a concentration from 0.1 to 10 weight percent of the organic solvent.

#### References Cited

##### UNITED STATES PATENTS

|    |           |         |                 |          |
|----|-----------|---------|-----------------|----------|
| 30 | 1,966,915 | 7/1934  | Baier           | 252—104  |
|    | 2,749,313 | 6/1956  | Williams et al. | 252—104  |
|    | 2,886,532 | 5/1959  | Hale et al.     | 8—111 X  |
|    | 2,914,374 | 11/1959 | Harris et al.   | 8—111    |
|    | 3,355,385 | 11/1967 | Macklet         | 202—10 X |

##### OTHER REFERENCES

McCutcheons—Detergents and Emulsifier, 1967, p. 255.

MAYER WEINBLATT, Primary Examiner

U.S. Cl. X.R.

8—111, 139, 142; 252—321